# EUROPEAN PATENT SPECIFICATION

(11) **EP 0 042 995 B1**
(45) Date of publication and mention of the grant of the patent: **15.05.1985**
(21) Application number: 81104301.7
(22) Date of filing: 04.06.1981
(51) Int. Cl.: B22D 11/00, B22D 11/04, B22D 11/14

(54) **Apparatus and method for continuous casting of metallic strands at exceptionally high speeds using oscillating mold assembly**
Einrichtung und Verfahren zum Stranggiessen metallischer Litze bei aussergewöhnlich hohen Geschwindigkeiten unter Verwendung einer oszillierenden Formeinrichtung
Appareil et procédé pour la coulée continue de fils métalliques à des vitesses exceptionnellement élevées utilisant un moule oscillant

(30) Priority: 09.06.1980 US 157933
(43) Date of publication of application: 06.01.1982
(73) Proprietor: KENNECOTT CORPORATION, Stamford Connecticut 06904 (US)
(72) Inventor: Shinopulos, George, Burlington, Mass. 01803 (US); Randlett, Ronald, Burlington, Mass. 01803 (US); Bower, Terry F., Needham, Mass. 02194 (US)
(74) Representative: Hoeger, Stellrecht & Partner

## Description

This invention relates to a method for continuously upcasting a metallic strand from a metallic melt comprising: providing a vertically oriented die having an inlet end with a coolerbody having a free end portion surrounding a portion of said die to enable portions of said die to be cooled and with an insulating member located within a recess in the coolerbody and between a portion of said die and a portion of said coolerbody to insulate a portion of said die from the cooling of said coolerbody, the inlet end of said die extending substantially below the free end portion of said coolerbody, and the location of said insulating member being at the free end portion of the coolerbody extending between said die and said coolerbody a predetermined distance, immersing said free end portion of said coolerbody into the melt a distance greater than said predetermined distance to produce a solidification front within the die when the melt is withdrawn through said coolerbody, withdrawing molten metal from the melt through said die while cooling said die through said coolerbody, said cooling completely solidifying the molten metal into a strand within a portion of the die above the insulating member, and providing alternating forward and reverse movements of the die and the strand relative to each other in a direction parallel to the direction of the travel of the strand, and to an apparatus carrying through this method.

An up-casting method and apparatus, resp., of this general type is known from EP-A -1-0 007 581. According to the known method alternating forward and reverse movements are caused in the solidified strand by withdrawal means operating on a controlled basis such that with the die having a fixed position forward and reverse strokes are generated in the strand, preferably with a dwell period between a reverse stroke and the next following forward stroke. It has been found that this type of operation is not completely satisfactory in some cases because, in order to achieve a fast reversal of the strand, heavy drive means are necessary for the withdrawal means.

Other methods of casting indefinite lengths of metallic strands, from a melt by drawing the melt through a cooled mold are also known. The mold generally has a die of a refractory material such as graphite cooled by a surrounding water jacket. US―A―3,354,936, for example, describes a cooled mold assembly sealed into the bottom wall of the melt container to downcast large billets. The force of gravity feeds the melt through the mold. In downcasting, however, there is a danger of a melt "break out" and the melt container must be emptied or tilted to repair or replace the mold or the casting die.

Horizontal casting through a chilled mold has also been tried. Besides the break out and replacement problems of downcasting, gravity can cause non-uniform solidification, resulting in a casting that is not cross-sectionally uniform or having an inferior surface quality.

Finally, various other arrangements have been used for upcasting. Early efforts are described in US-A-25 53 921 and US-A-21 71 132. US-A-25 53 921 employs a water cooled, metallic "mold pipe" with an outer ceramic Edng that is immersed in a melt. In practice, no suitable metal has been found for the mold pipe, the casting suffers from uneven cooling, and condensed metallic vapors collect in a gap between the mold pipe and the liner due to differences in their coefficients of thermal expansion. US―A―21 71 132 also uses a water-cooled "casing", but it is mounted above the melt and a vacuum is required to draw melt up to the casting. A coaxial refractory extension of the casing extends into the melt. The refractory extension is necessary to prevent "mushrooming", that is, the formation of a solid mass of the metal with a diameter larger than that of the cooled casing. In both cases thermally generated gaps, in this instance between the casing and the extension, can collect condensed metal vapor which results in poor surface quality of termination of the casting.

US-A-37 46 077 and US-A-38 72 913 more recent upcasting apparatus and techniques. The second patent avoids problems associated with thermal expansion differences by placing only the tip of a "nozzle" in the melt. A water-cooled jacket encloses the upper end of the nozzle. Because the surface of the melt is below the cooling zone, a vacuum chamber at the upper end of the nozzle is necessary to draw the melt upwardly to the cooling zone. The presence of the vacuum chamber, however, limits the rate of strand withdrawal and requires a seal.

US―A―37 46 077 avoids the vacuum chamber by immersing a cooling jacket and a portion of an enclosed nozzle into the melt. The immersion depth is sufficient to feed melt to the solidification zone, but it is not deeply immersed. The jacket, as well as the interfaces between the jacket and the nozzle, are protected against the melt by a surrounding insulating lining. The lower end of the lining abuts the lower outer surface of the nozzle to block a direct flow of the melt to the cooling jacket.

The foregoing systems are commonly characterized as "closed" mold, in that the liquid metal communicates directly with the solidification front. The cooled mold is typically fed from an adjoining container filled with the melt. In contrast, an "open" mold system feeds the melt, typically by a delivery tube, directly to a mold where it is cooled very rapidly. Open mold systems are commonly used in downcasting large billets of steel, and occasionally aluminium, copper or brass. However, open mold casting is not used to form products with a small cross section because it is very difficult to control the liquid level and, hence, the location of the solidification front.

A problem that arises in closed mold casting is a thermal expansion of the bore of the casting die between the beginning of the solidification front and the point of complete solidification termed "bell-mouthing". This condition results in the formation of enlargements of the casting cross section which wedge against a narrower portion of the die. The wedged section can break off and form an immobile "skull". The skulls can either cause the strand to terminate or can lodge on the die and produce surface defects on the casting. Therefore, it is important to maintain the dimensional uniformity of the die bore within the casting zone. According to US-A-38 72 913 and US―A―37 46 077 these problems are controlled by a relatively gentle vertical temperature gradient along the nozzle due in part to a modest cooling rate to produce a generally flat solidification front. With this gentle gradient, acceptable quality castings can be produced only at a relatively slow rate, typically five to forty inches per minute.

Another significant problem in casting through a chilled mold is the condensation of metallic vapors. Condensation is especially troublesome in the casting of brass bearing zinc or other alloys bearing elements which boil at temperatures below the melting temperature of the alloy. Zinc vapor readily penetrates the materials commonly used to form casting dies, as well as the usual insulating materials, and can condense to liquid in critical regions. Liquid zinc on the die near the solidification front can boil at the surface of the casting, resulting in a gassy surface defect. Because of these problems, present casting apparatus and techniques are not capable of commercial production of good quality brass strands at high speeds.

The manner in which the casting is drawn through the chilled mold is also an important aspect of the casting process. A cycled pattern of a forward withdrawal stroke followed by a dwell period, is used commercially in conjunction with the mold unit described in the aforementioned US-A-38 72 913. US-A-39 08 747 discloses a controlled reverse stroke to form the casting skin, prevent termination of the casting, and compensate for contraction of the casting within the die as it cools. GB-A-10 87 026 also discloses a reverse stroke to partially remelt the casting. US-A-33 54 936 discloses a pattern of relatively long forward strokes, followed by periods where the casting motion is stopped and reversed for a relatively short stroke. This pattern is used in downcasting large billets to prevent inverse seg- ration. In all of these systems, however, the stroke velocities and net casting velocities are slow. In this '936 system, for example, forward strokes are three to twenty seconds in duration, reverse strokes are one second in duration, and the net velocity is thirteen to fifteen inches per minute.

It is known to oscillate a continuous casting mold to provide stripping action to facilitate the movement of the newly cast rod through the mold and more importantly, when the rate of advancement of the mold during a portion of the cycle is greater than that of the rod being cast, to prevent tension tears in the solidifying skin. Moreover, creating the casting strokes by mold oscillation allows the rod to be withdrawn from the mold at a constant rate, thereby facilitating further processing operations after casting, for example, the conversion of rod to strip.

Proceeding on the basis of the prior art according to the above referenced EP-A-0 007 581 it has to be regarded as the object underlying the present invention to avoid the rather complicated and energy-consuming reversal of the drive means for the strand and to achieve the intended relative movement between the die and the strand in a more favourable manner.

This object is accomplished according to the invention in that the solidified strand is withdrawn from said melt at a constant rate, and that said die is oscillated in a direction parallel to the direction of travel of said strand.

A preferred apparatus for continuously up- casting a metallic strand from a metallic melt according to this method comprises: a vertically oriented, generally tubular die having an inlet end for fluid communicatibn with the melt, a coolerbody having a free end portion surrounding a portion of said die to enable portions of said die to be cooled the inlet end of said die extending substantially below the free end portion of said coolerbody, an insulating member located between a portion of said die and said coolerbody to insulate a portion of said die from the cooling of said coolerbody, the location of said insulating member being at said free end portion of the coolerbody and extending between said die and said coolerbody a predetermined distance, supporting means mounted for immersing said free end portion of said coolerbody in the melt a distance greater than said predetermined distance to produce a solidification front within the die below the level of the melt when the melt and the solidified strand is withdrawn through said die, means for withdrawing the melt and the strand through said die while cooling said die through said coolerbody, said cooling completely solidifying the molten metal into said strand within a portion of the die below the level of the melt and above the insulating member, this apparatus according to the invention being characterized in that the solidified strand is withdrawn from said melt at a constant rate by the withdrawing means, and that oscillating means are provided for oscillating said die in a vertical direction parallel to the direction of travel of said strand in a pattern of forward and reverse strokes.

Preferably a mold assembly of this invention oscillates in substantially the same direction as the rod being cast with little or not lateral movement.

An inventive mold assembly accommodates a steep temperature gradient along a casting die, particularly at the lower end of a solidification zone, without the formation of skulls or loss of dimensional uniformity in the casting zone.

Consequently, it is possible to produce high quality strands at exceptionally high speeds.

Further, a mold assembly according to the invention having the foregoing advantages that, has a relatively low cost of manufacture, is convenient to service and is durable.

Preferably an oscillating cooled mold assembly for continuous high-speed casting of metf'iic strands has a hollow die formed of a refractory material. A melt, typically of copper or copper alloys such as brass, is in fluid communication with one end of the die. A coolerbody, preferably water-cooled, encloses the die, preferably in a tight-fitting relationship. The coolerbody preferably has a high cooling rate that produces a solidification front within a casting zone of the die spaced from the die end adjacent the melt. Means are provided for drawing the melt through the mold assembly to effect solidification of a rod or strand. The mold assembly is supported for oscillation in a direction substantially parallel to the direction of travel of the rod through the mold, and. the means by which the mold assembly is caused to oscillate as the rod or strand advances creates the effect of both upward and downward casting strokes. By oscillating the mold while withdrawing the rod or strand at a constant velocity, the relative motion between mold and rod is controllable over a wide range. Means are provided to deliver coolant to the chilled mold during oscillation.

In a preferred embodiment of the invention, a coolant manifold extension assembly communicates with, and supplies coolant to, the coolerbody. The manifold extension assembly in turn attaches to a support manifold which supplies the extension assembly with coolant. An insulating hat surrounds the coolerbody and manifold ex- - tension assembly, thermally insulating them from the metallic melt. The insulating hat attaches the support manifold by spring biased mounting means. The manifold extension assembly features three concentric tubes forming two annular elongated passageways therebetween, with one of the annular passageways being adapted for supplying coolant to the coolerbody, and the other passageway being adapted for receiving the coolant from the coolerbody. The two inner tubes fit slidably into 0-ring gland seals in the support manifold.

The means for accomplishing mold oscillation may include at least one hydraulic actuator controlled by a servo valve and computer means. Mold oscillation wave forms can be shaped to provide unlimited variation in stripping velocity, return velocity and dwell. This is extremely useful in determining optimum mold motion programs for different casting alloys.

The die preferably has a longitudinally uniform cross section. It can have a slight upwardly narrowing taper or stepped configuration on its inner surface. The die is preferably slip fit into the coolerbody to facilitate replacement. Before the die expands thermally against the coolerbody, it is restrained against axial movement by a slight upset in the mating coolerbody wall near the top and a stepped outer surface that engages the lower face of the coolerbody. Also, in the preferred form a metallic foil sleeve is interposed between the outside insulating member and the counterbore to facilitate removal of the insulator.

The coolerbody preferably has a double wall construction with an annular space between the walls. The inner wall adjacent the die is preferably formed from a sound ingot of age hardened chrome copper alloy; the outer sleeve is preferably formed of stainless steel. The inner and outer walls or "bodies" are preferably bonded at their lower ends by a copper/gold braze joint. Water is typically circulated in a temperature range and flow rate that yields a high cooling rate of the melt advancing through the die while avoiding condensation of water vapor on the mold assembly or the casting. A vapor shield and gaskets are preferably disposed between the immersed end of the coolerbody and the surrounding insulating hat.

These and other objects and features of the invention will become apparent to those skilled in the art from the following detailed description which should be read in light of the accompanying drawings.

### Brief Description of the Drawings

Fig. 1 is a simplified view in perspective of a strand production facility that employs oscillating mold assemblies and methods embodying the present invention;
Fig. 2 is a side view partially in section of the oscillating mold and supporting structure in conjunction with a furnace for holding a melt;
Fig. 3 is a perspective view of the structure for supporting the oscillating mold;
Fig. 4 is an isolated sectional view of the support manifold extension assembly and mold of the structure of Fig. 2;
Fig. 5 is an enlarged view of the coolerbody and mold of the structure of Fig. 4;
Fig. 6 is a top plan view of the coolerbody shown in Fig. 5;
Figs. 7-9 are diagrammatic representations of the position of the mold in a melt during various stages of mold oscillation;
Fig. 10 is a simplified views in vertical section showing the casting furnace shown in Fig. 1 in its lower and upper limit positions with respect to the mold assemblies;
Figs. 11 and 12 are simplified views in vertical section of alternative arrangements for controlling the expansion of the die below the casting zone;
Fig. 13 is a perspective view of the carriage which supports a mold for oscillation;
Fig. 14 is an isolated plan view of the carriage assembly of the structure of Fig. 2 for supporting and moving the oscillating mold; and
Fig. 15 is a side elevational view, in section, of the carriage assembly of Fig. 14.

### Detailed Description of the Preferred Embodiments

Fig. 1 shows a suitable facility for the continuous production of metallic strands in indefinite lengths by upwardly casting the strands through cooled molds according to this invention. Four strands 12 are cast simultaneously from a melt held in a casting furnace 16. The strands, which can assume a variety of cross sectional shapes such as square or rectangular, and diameters will be described as rods having a substantially circular cross section with a diameter in the range of one quarter to two inches.

With reference to Fig. 1, the strands 12 are cast in four cooled mold assemblies 18 mounted on four vertically movable carriage assemblies 20. A withdrawal machine 22 draws the strands at a constant rate through the mold assemblies and directs them to a pair of booms 24, 24' that guide the strands to four pouring type coilers 26 where the strands are collected in coils. Each boom 24 is hollow to conduct cooling air supplied by the ducts 28 along the length of the boom.

The melt is produced in one or several melt furnaces (not shown) or in one combination melting and holding furnace (not shown). While this invention is suitable for producing continuous strands formed from a variety of metals and alloys, it is particularly directed to the production of copper alloy strands, especially brass. A ladle 30 carried by an overhead crane (not shown) transfers the melt from the melt furnaces to the casting furnace 16. The ladle preferably has a tea- pot-type spout which delivers the melt with a minimum of foreign material, such as cover and dross. To facilitate the transfer, the ladle is pivotally seated in support cradle 32 on a casting platform 34. A ceramic pouring cup 36 funnels the melt from the ladle 30 to the interior of the casting furnace 16. The output end of the pouring cup 36 is located below the casting furnace cover and at a point spaced from the mold assemblies 18. In continuous production, as opposed to batch casting, additional melt is added to the casting furnace when it is approximately half full to blend the melt both chemically and thermally.

The casting furnace is supported on a hydraulic, scissor-type elevator and dolly 38 that includes a set of load cells 38a (Fig. 10) to sense the weight of the casting furnace and its contents. Output signals of the load cells 38a are conditioned to control the furnace elevation; this allows automatic control of the level of the melt with respect to the coolerbody. As is best seen in Fig. 10, the casting furnace is movable between a lower limit position in which the mold assemblies 18 are spaced above the upper surface of the melt 14 when the casting furnace is filled and an upper limit position (shown in phantom) in which the mold assemblies are adjacent the bottom of the casting furnace. The height of the casting furnace is continuously adjusted during casting to maintain the selected immersion depth of the mold assemblies 18 in the melt. In the lowered position, the mold assemblies are accessible for replacement or servicing, after the furnace is rolled out of the way.

It should be noted that this production facility usually includes back-up level controls such as probes, floats, and periodic manual measurement as with a dunked wire. These or other conventional level measurement and control systems can also be used instead of the load cells as the primary system. Also, while this invention is described with reference to fixed mold assemblies and a movable casting furnace, other arrangements can be used. The furnace can be held at the same level with melt added periodically or continuously to maintain the same level. Another alternative includes a very deep immersion so that level control is not necessary. A significant advantage of this invention is that it allows this deep immersion. Each of these arrangements has advantages and disadvantages that are readily apparent to those skilled in the art.

The casting furnace 16 is a 96.5 cm coreless induction furnace with a rammed alumina lining heated by a power supply. A furnace of this size and type can hold approximately five tons of melt. The furnace 16 has a pouroff spout 16a that feed to an overfill and pouroff ladle 42 (Fig. 10).

Referring again to Fig. 1, the withdrawal machine 22 has four opposed pairs of pinch rolls 44 that each frictionally engage one of the strands 12. The pinch rolls 44 are secured on a common shaft driven by a servo-controlled, reversible hydraulic motor 46. A conventional variable-volume, constant-pressure hydraulic pumping unit that generates pressures of up to 210 bar drives the motor 46. A conventional electronic programmer (not shown) produces a program of signals that controls the operation of the motor 46 through a conventional servo system. The program includes a programmed start-up routine that gradually ramps up the withdrawal speed. The drive rolls 44 can be individually disengaged from a selected strand 12 without interrupting the advance of the other strands.

Referring now to Fig. 2, a mold assembly 18 is immersed in a melt 14 contained by a furnace 16. Fig. 2 shows a protective cone 48 which melts away after the assembly 18 is immersed in the melt 14. The protective cone 48 is normally formed of copper and takes less than one minute to completely dissolve. The purpose of the protective cone is to prevent dross and other impurities from entering a die 112 upon immersion. Once the assembly is immersed in the melt and the cone has disintegrated, molten metal is drawn through the assembly 18. Initially, the process is started by inserting a solid starter rod (with a bolt on the end of it) through the die 112 from the upper part of the assembly into the melt. Molten metal solidifies on the bolt and, when the rod is pulled through the die 112, the molten metal follows, solidifying on its way. After a solidified rod or strand 12 has been threaded through pinch rolls 44, the starter rod (with a small piece of the strand 12) is severed from the remainder of the strand 12. Once the strand 12 has been formed from the melt 14, it is continuously withdrawn at a constant speed by one or more pairs of the pinch rollers 44. Thus, the strand 12 continuously advances away from the melt at a constant velocity, generally in the range of from 508 to 1016 cm/min in the direction shown by an arrow 52. While the strand 12 is advancing, the entire assembly 18 oscillates in the vertical direction. Basically, the assembly 18 is connected to a carriage assembly 20 for controlled oscillation in the range of 12 to 150 cycles per minute.

As the chilled mold assembly 18 oscillates, it is cooled by means of a coolant supplied to a manifold 54 mounted to the carriage assembly 20 through flexible tubes 56. The coolant delivery system is specifically described in conjunction with Figs. 4 and 5.

It should be pointed out that although the production facility of Fig. 1 makes use of four independently oscillating mold assemblies 18 to produce the four strands 12, any other number of mold assemblies may be used in tandem, as dictated by specific production requirements.

Because the mold assembly 18 oscillates during the casting process, high dynamic loads develop which must be accommodated by the supporting structure. The superstructure which resists these loads with a minimum of deflection, will now be described in detail in conjunction with Figs. 2 and 3. Referring first to Fig. 3, the overall supporting structure is a rigid steel box. The vertical loads are supported by the columnar structural members 58, 60, 62, 64 which are steel I-beams. The columnar members 58, 60, 62, 64 are tied together by the horizontal steel I-beams 66, 68, 70 and 72. The horizontal members 66, 68, 70, 72 and 74 are preferably welded to the columnar members 58, 60, 62 and 64. The horizontal I-beams 66, 68 and 70 are oriented so that their flange faces extend in the vertical direction for maximum stiffness in carrying the oscillation induced loads. The beams 72 and 74 are further stiffened respectively by angle pieces 72a and 74a welded to the beams. The beams 66 and 70 are stiffened in the vertical direction by bracing means 75, 76, 78 and 80, which are also made of steel. Steel beams 82 and 84 further strengthen the structure at its bottom.

The carriage structure is mounted to angle pieces 72a and 74a which totally support the carriage through horizontal I-beams 72 and 74. Carriage load paths are fed to the frame base through beams 86, 88, 78, 80, 75 and 76. The steel I-beams 89 and 90 are welded between the horizontal beams 68 and 72. These beams 89 and 90 support the oscillating carriage supporting superstructure comprising vertical I-beams 91 and 92 and horizontal I-beams 93, 94 and 95. The beams 93 and 95 are welded to the steel I-beam 74 which connects the columnar beams 60 and 64 at their tops. The structure is rendered more rigid by bracing steel I-beams 86 and 88.

The carriage assembly 20 (Fig. 2) is shown in greater detail in Fig. 13. This assembly 20 is constructed of steel angle plates 201 and 202 welded to bottom plate 203 and back plate 205. A top plate 207 is welded to the back plate 205 and the angle plates 201 and 202 to complete the structure. The plates 201 and 202 approximately 2.5 cm thick, are lightened by means of holes 209 and 210 respectively.

The carriage assembly 20 supports the manifold 54 (Fig. 2) by means of bolts through the bolt holes 211a (Fig. 13) which encircle a hole 213 in the bottom plate 203. The hole 213 allows the cast strand to pass through on its way to the pinch rollers 44 (Fig. 2).

Referring now to Figs. 13 and 14, the carriage assembly 20 is constrained to move in the vertical direction by rails 215. These rails 215 are spaced apart from the angle plates 201 and 202 by means of spacers 217. The rails 215 and spacers 217 are bolted and doweled to the angle plates 201 and 202.

The rails 215 have beveled edges which closely engage beveled idler rollers 219 (Fig. 14). The rollers 219 are bolted to structural assembly 221. The structural assembly 221 includes welded box structures 223 for added rigidity. The structural assembly 221 is bolted rigidly to the superstructure described above in reference to Fig. 3.

With reference to Figs. 14 and 15, the carriage assembly 20 is supported for oscillation in the vertical direction by hydraulic cylinder 225. The piston within the hydraulic cylinder 225 attaches to the top plate of carriage assembly 20 by means of bracket 227. The hydraulic cylinder 225 is controlled by servo valve 229 through manifold block 231.

The hydraulic cylinder 225 itself is supported by arms 233 (Fig. 14) which are bolted to the structural assembly 221. The servo valve 229 is under the control of a computer (not shown) which commands the desired relative motion between strand and mold for proper solidification of the cast strand. In particular, mold oscillation will create the same effect with respect to the rod or strand 12 as a pattern of forward and reverse strokes of the rod or strand itself.

Figs. 7-9 are provided to show the effect of mold oscillation on casting skin formation and to provide reference for the terms "upward" and "downward" strokes. Fig. 7 shows the mold assembly 18 at its lowest point in the melt 14. At this instant in time, the mold assembly would be just beginning its acceleration in the upward direction as is indicated by the small arrow 41. At this time, the upward velocity of the strand would be greater than the upward or forward velocity of the mold. It should be noted that the solidification skin 12a of strand 12 is very thin. Fig. 8 shows the mold assembly 10 at about the middle of its travels up and down the melt. By the time the mold assembly has reached mid-point, its upward velocity is greater than the upward velocity of the strand. This is due to an acceleration of the mold assembly in the upward direction which is about 2 g for most applications. It is again emphasized that the velocity of the strand is constant, and only the velocity of the mold assembly varies. In Fig. 8 a solidification front 29 has moved near the top of the melt. Skin 12a is thicker as opposed to the skin shown in Fig. 7.

Fig. 9 shows the mold at the top of its path of travel. At the particular instant depicted in Fig. 9, the mold velocity in the upward or forward direction is zero and is about to begin its trip back down to the position shown in Fig. 7. At this position, the solidification skin 12a is thickest. Upward and downward speeds are separately settable in the computer to obtain optimum surface quality and material structure. In view of Figs. 7-9 it should be apparent that the term "upward stroke" refers to the movement of the mold assembly away from the melt while the term "downward stroke" refers to the movement of the mold assembly further into the melt.

Figs. 4 and 5 show a preferred embodiment of the mold assembly 18 and illustrate how coolant is supplied continuously thereto. Coolant, preferably water, enters the manifold 54 at an inlet 100 and travels down an annular passageway 101 in a manifold extension assembly 102 and continues into a coolerbody 103 to cool a mold 104. The coolant returns through an annular passageway 105 and out an outlet 106. The passageways 101 and 105 are the annular spaces created by three concentric tubes 107, 108 and 109, each formed of steel. The outer tube 107 is flange mounted to the manifold 54. The two inner tubes 108 and 109 slide into 0-ring gland seals 110 in manifold 54. By this arrangement, dimensional changes caused by thermal gradients are accommodated.

The concentric tube design for the manifold extension assembly 102 permits high coolant flow rates while minimizing the cross sectional area of the assembly which must oscillate within the furnace melt. Minimizing the cross sectional area is important in holding down the hydrodynamic loading on the oscillating mold assembly.

Referring now to the great detail of Fig. 5, a tubular die 112 is enclosed by the coolerbody 103. The die 112 has a lower end portion 112a that projects beyond the lower face 103a of the coolerbody. The die portion 112a and at least a portion of the coolerbody are immersed in the melt 14 during casting. Cuprostatic pressure forces liquid melt into the die toward the coolerbody. On start up, a length of straight rod is inserted into the die through a graphite plug and positioned with its lower end, which typically holds a bolt, somewhat above a normal solidification or casting zone 114. The immersion depth is selected so that the liquid melt reaches the casting zone 114 where rapid heat transfer from the melt to the coolerbody solidifies the melt to form a solid casting without running past the starter rod. The melt adjacent the die will cool more quickly than the centrally located melt so that an annular "skin" forms around a liquid core. The liquid solid interface defines a solidification front 114a across the casting zone 114. It is preferred that the peak of solidification front 114a be always located beneath the surface of melt 14. Since solidification initiates within the area of die 112 backed by insulating bushing 118, the location of the solidification front is well defined. A principal feature of this invention is that the casting zone is characterized by a high cooling rate and a steep vertical temperature gradient at its lower end so that it extends over a relatively short length of the die 112. These features are a result of initiating solidification of the melt within the area of the die backed by the insulating member or bushing 118.

The die 112 is formed of a refractory material that is substantially non-reactive with metallic and other vapors present in the casting environment especially at temperatures in excess of 1093°C. Graphite is the usual die material, although good results have also been obtained with boron nitride. More specifically, a graphite sold by the Poco Graphite Company under the trade designation DFP-3 has been found to exhibit unusually good thermal characteristics and durability. Regardless of the choice of material for the die, before installation it is preferably outgassed in a vacuum furnace to remove volatiles that can react with the melt to cause start-up failure or produce surface defects on the casting. The vacuum environment also prevents oxidation of the graphite at the high outgassing temperatures, e.g. 399°Cfor 90 minutes in a roughing pump vacuum. It will be understood by those skilled in the art that the other components of the mold assembly must also be freed of volatiles, especially water prior to use. Components formed of "Fiberfrax" refractory material (the registered trade mark of the Carborundum Co. for alumina silica refractory paper material) are pretreated by heating to about 816°C; other components such as those formed of silica are typically heated from 177 to 204°C.

The die 112 has a generally tubular configuration with a uniform inner bore diameter and a substantially uniform wall thickness. The inner surface of the die is highly smooth to present a low frictional resistance to the axial or longitudinal movement of the casting through the die and to reduce wear. The outer surface of the die, also smooth, is pressure contacted with the surrounding inner surface 103b of the coolerbody 103 during operation. The surface 103b constrains the die as it attempts to expand radially due to heating by the melt and the casting, and promotes a highly efficient heat transfer from the die to the coolerbody by the resulting pressure contact.

The fit between the die and the coolerbody is important since a poor fit, one leaving gaps, severely limits heat transfer from the die to the coolerbody. A tight fit is also important to restrain longitudinal movement of the die with respect to the coolerbody due to friction or "drag" between the casting and the die as the casting is drawn through the die. On the other hand, the die should be quickly and conveniently removable from the coolerbody when it becomes damaged or worn. It has been found that all of these objectives are achieved by machining the mating surfaces of the die and coolerbody to close tolerances that permit a "slip fit" that is, an axial sliding insertion and removal of the die. The dimensions forming the die and mating surface 103b are selected so that the thermal expansion of the die during casting creates a tight fit. While the die material typically has a much lower thermal expansion coefficient than the coolerbody, the die is much hotter than the coolerbody so that the temperature difference more than compensates for the differences in the thermal expansion coefficients. The average temperature of the die in the casting zone through its thickness is believed to be approximately 538°C for a melt at 1093°C. The coolerbody is near the temperature of the coolant, usually 27 to 38°C, circulating through it.

Mechanical restraint is used to hold the die in the coolerbody during low speed operation or set-up prior to it being thermally expanded by the melt. A straightforward restraining member such as a screw or retainer plate has proven impractical because the member is cooled by the coolerbody and therefore condenses and collects metallic vapors. This metal deposit can create surface defects in the casting and/or weld the restraining member in place, which greatly impedes replacement of the die. Zinc vapor present in the casting of brass is particularly troublesome. An acceptable solution is to create a small upset or irregularity 103c on the inner surface 103b of the coolerbody, for example, by raising a burr with a nail set. A small step 116 formed on the outer surface of the die which engages the lower face 103a of the coolerbody (or more specifically, an "outside" insulating bushing or ring 118 seated in counterbore 103d formed in the lower end of the coolerbody) indexes the die for set-up and provides additional upward constraint against any irregular high forces that may occur such as during start-up. It should also be noted that the one-piece construction of the die eliminates joints, particularly joints between different materials, which can collect condensed vapors or promote their passage to other surfaces. Also, a one-piece die is more readily replaced and restrained than a multi-section die.

Alternative arrangements for establishing a suitable tight-fitting relationship between the die and coolerbody include conventional press or thermal fits. In a press fit, a molybdenum sulfide lubricant is used on the outside surface to reduce the likelihood of fracturing the die during press fitting. The lubricant also fills machining scratches of the die. In the thermal fit, the coolerbody is expanded by heating, the die is inserted and the close fit is established as the assembly cools. Both the press fit and the thermal fit, however, require that the entire mold assembly 18 be removed from the cooling water manifold to carry out the replacement of a die. This is clearly more time consuming, inconvenient and costly than the slip fit.

While the preferred form of the invention utilizes a one-piece die with a uniform bore diameter, it is also possible to use a die with a tapered or stepped inner surface that narrows in the upward direction, or a multisection die formed of two or more pieces in end-abutting relationship. Upward narrowing is desirable to compensate for contraction of the casting as it cools. Close contact with the casting over the full length of the die increases the cooling efficiency of the mold assembly. Increased cooling is significant because it helps to avoid a central cavity caused by an unfed shrinkage of the molten center of the casting.

To minimize expense, an opposite taper can be machined on the outer surface of the die rather than on its inside surface, or the inside surface 103b of the coolerbody. Thermal expansion of the die within the coolerbody bore during casting creates the desired upwardly narrowing taper on the highly smooth inner surface of the die. Multi- section dies can either have the same bore diameter or different bore diameters to create a stepped upward narrowing. To avoid troublesome accumulations of metal between the die sections, junctions between sections should occur only above the casting zone. Also, the upper section or sections above the casting zone can be press fit since the lower section is the most likely to become damaged and need replacement.

By way of illustration, but not of limitation, a one-piece die formed of graphite, suitable for casting 19 mm rod, has a length of approximately 26.7 cm and a uniform wall thickness of approximately 3 to 5 mm. In general, the wall thickness will vary with the diameter of the casting. The projecting die portion 112a typically has a length of 5cm.

The coolerbody 103 has a generally cylindrical configuration with a central, longitudinally extending opening defined by the inner surface 103b. The interior of the coolerbody has a passage designated generally at 120 that circulates the cooling fluid, preferably water, through the coolerbody. A series of coolant inlet openings 120a and coolant outlet openings 120b are formed in the upper end of the coolerbody. As is best seen in Fig. 6, these openings are arrayed in concentric circles with sufficient openings to provide a high flow rate, typically 3.8 I pro 454 of casting per minute. A pair of 0-rings 122 and 123, preferably formed of a long wearing fluoroelastomer, seal the manifold extension assembly 102 (see Fig. 5) in fluid communication with the inlet and outlet openings. A mounting flange 124 on the coolerbody has openings 124a that receives bolts (not shown) to secure the mold assembly to-the manifold extension assembly. This flange also includes a hole (not shown) to vent gases from the annular space between the coolerbody and an insulating hat (see Fig. 4) through a tube (not shown) in the manifold 54 to atmosphere.

The coolerbody has four main components: an inner body 126, an outer body 128, a jacket closure ring 130 and the mounting flange 124. The inner body is formed of alloy that exhibits excellent heat transfer characteristics, good dimensional stability and is hard and wear resistant. Age hardened copper such as the alloy designated CDA 182 is preferred. The outer body 128, closure ring 130 and mounting flange 124 are preferably formed of stainless steel, particularly free machining 303 stainless for the ring 130 and flange 124, and 304 stainless for the outer body 128. Stainless exhibits satisfactory resistance to mechanical abuse, possesses similar thermal expansion characteristics as chrome copper, and holds up well in the casting environment. By the use of stainless steel, very large pieces of age hardened copper are not required, thus making manufacture of the coolerbody more practical.

The inner body is machined from a single cylindrical billet of sound (crack-free) chrome copper. Beside cost and functional durability advantages, the composite coolerbody construction is dictated by the difficulty in producing a sound billet of chrome copper, which is large enough to form the entire coolerbody. Longitudinal holes 120c are deep drilled in the inner body to define the inlets 120a. The holes 120c extend at least to the casting zone and preferably somewhat beyond it as shown in Fig. 5. Cross holes 120d are drilled to the bottom of the longitudinal holes 120c. The upper and lower ends of the inner body are threaded at 126a and 126b to receive the mounting flange 124 and the closure ring 130, respectively, for structural strength. The closure ring has an inner upwardly facing recess 130a that abuts a mating step machined on the inner body for increased braze joint efficiency, to retard the flow of cooling water into the joint, and to align the ring with the inner body. An outer, upwardly facing recess 130b seats the lower end of the outer body 128 in a fluid-tight relationship.

Because the threaded connection at 126b will leak if not sealed well and is required to withstand resolutionizing and aging of softened coolerbody bores, the joint is also copper/gold brazed. While copper/gold brazing is a conventional technique, the following procedures produce a reliable bond that holds up in the casting environment. First, the mating surfaces of the closure ring and the inner body are copper plated. The plating is preferably 0.025 to 0.054 mm thick and should include the threads, the recess 130a and groove 130c. The braze material is then applied, as by wrapping a wire of the material around the inner body in a braze clearance 126c above the threads and in the groove 130c atop closure ring 130.

Two turns of a 1.6 mm diameter wire that is sixty percent copper and forty percent gold is recommended in clearance 126c and three turns in groove 130c. A braze paste of the same alloy is then spread over the mating surfaces. The closure ring is tightly screwed onto the inner body and the assembly is placed in a furnace, brazed end down, and preferably resting on a supported sheet of alumina silica refractory paper material such as the product sold by Carborundum Co. under the registered trade mark "Fiberfrax". The brazing temperature is measured by a thermocouple resting at the bottom of one of the longitudinal holes 120c. The furnace brings the assembly to a temperature just below the fusing point of the braze alloy for a short period of time such as 960 to 977°C for ten minutes. The furnace atmosphere is protected (inert or a vacuum) to prevent oxidation. The assembly is then rapidly heated to a temperature that liquifies the braze alloy (1016 to 1038°C) and is immediately allowed to cool to room temperature, again in a protected atmosphere. Solution treating of the chrome copper is best performed at a separate second step, by firing the part to 932 to 954°C for 15 minutes in a protected atmosphere and followed by liquid quenching.

Once the closure ring is joined to the inner body, the remaining assembly of the coolerbody involves TIG welding type 304 to type 303 stainless steel using type 308 rod after preheating parts to 204°C. The outer body 128, which has a generally cylindrical configuration, is welded at 134 to the closure ring.

The upper end of the outer body has an inner recess 128a that mates with the mounting flange 124 just outside the water outlet openings 120b. A weld 136 secures those parts. The closure ring and mounting flange space the outer body from the inner body to define an annular water circulating passage 120e that extends between the cross holes 120d and the outlet openings 120b. A helical spacer 138 is secured in the passage 120e to establish a swirling water flow that promotes a more uniform and efficient heat transfer to the water. The spacer 138 is preferably formed of 6 mm copper rod. The spacer coil is filed flat at points 138a to allow clearance for holding clips 140 secured to the inner body. A combination aging (hardening) treatment of the chrome copper and stress relief of the welded stainless steel is accomplished at 482°C for at least two hours in a protected atmosphere. The coolerbody is then machined and leak tested.

By way of illustration only, cooling water is directed through the inlets 120a, the holes 120c and 120d, and the spiral flow path defined by the passage 120e and the spacer 138 to the outlets 120b. The water is typically at 27 to 32°C at the inlet and heats approximately 6 to 12°C during its circulation through the coolerbody. The water typically flows at a rate of about 3.8 I per 454 g of strand solidified in the casting zone per minute. A typical flow rate is 95 per minute. The proper water temperature is limited at the low end by the condensation of water vapor. On humid days, condensation can occur at 21°C or below, but usually not above 27°C. Water temperatures in excess of 49°C are usually not preferred. It should be noted that the inlet and outlet holes can be reversed; that is, the water can be applied to the outer ring of holes 120b and withdrawn from the inner ring of holes 120a with no significant reduction in the cooling performance of the coolerbody. The spacing between the die and the inner set of holes is, however, a factor that affects the heat transfer efficiency from the casting to the water. For a 18 mm strand 12, the spacing is typically approximately 1.6 cm. This allows the inner body 126 to be rebored to cast a 2.54 cm diameter strand and accept a suitably dimensional outside insulator 118. In general, the aforedescribed mold assembly provides a cooling rate that is high compared to conventional water jacket coolers for chilled mold casting in closed systems.

Another important feature of this invention is the outside insulating bushing 118 which ensures that the die is dimensionally uniform in the casting zone and prevents an excessive outward expansion of the die below the zone (bell-mounting) that can lead to termination, start up defects, or surface defects. The bushing 118 is also important in creating a steep axial die temperature gradient immediately below the casting zone. For example, without the bushing 118, a sharp temperature gradient would exist at the entrance of the die into the coolerbody causing the lower portion 112a of the die to form a bell-mouth casting skin. The enlarged portion cannot be drawn into the co.olerbody past the casting zone. It wedges, breaks off from the casting, and can remain in place as casting continues. This wedged portion can result in poor surface quality or termination of the strand. The bushing 118 prevents this problem by mechanically restraining the outward expansion of the die immediately below the casting zone 114. It also insulates the die to a great extent from the coolerbody to create a gentle thermal gradient in the die over the region extending from the lower coolerbody face 103a to somewhat below the lower edge of the casting zone 114.

The bushing 118 is formed of a refractory material that has a relatively low coefficient of thermal expansion, a relatively low porosity, and good thermal shock resistance. The low coefficient of thermal expansion limits the outward radial pressures exerted by the bushing on the coolerbody and, with the coolerbody, constrains the graphite to maintain a substantially uniform die inner diameter. The low coefficient of thermal expansion also allows the bushing 118 to be easily removed from the coolerbody by uniformly heating and assembly to 121°C. A suitable material for the bushing 118 is cast silica glass (Si0₂) which is machinable.

The bushing 118 extends vertically from a lower end surface 118a that is flush with the lower coolerbody face 103a to an upper end surface 118b somewhat above the lower edge of the casting zone. In the production of three-quarter inch brass rod, a bushing having a wall thickness of approximately 6 mm and a length of 3.5 cm has yielded satisfactory results.

In practice, it has been found that metallic vapors penetrate between the inside insulating bushing 118 and the coolerbody counterbore 103d, condense and bond the ring to the coolerbody making it difficult to remove. A thin foil shim 142 of steel placed between the ring and the counterbore solves this problem. The bushing and the shim are held in the counterbore by a special thermal fit, that is, one which allows easy assembly and removal when the bushing and the coolerbod^{y} are heated to 204°C.

Figs. 11 and 12 illustrate alternative arrangements for ensuring that the casting occurs in a dimensionally uniform portion of the die and for controlling the expansion of the die below the casting zone. Fig. 11 shows a die 112' which is identical to the die 112, except that the projecting lower portion 112a has an upwardly expanding tapt-.- formed on its inner surface. The degree of taper is selected to produce a generally uniform diameter bore when the die portion expands in the melt. This solution, however, is difficult to fabricate. Also, in practice, it is nevertheless necessary to use the bushing 118 (shown in phantom) as well as the die 112' to achieve the high production speeds and good casting quality characteristics of this invention.

Fig. 12 shows an "inside" insulator 144 that slips inside a die 112" which is the same as the die 112 except that it is terminated flush with the coolerbody face 103a. The inside insulator 144 is formed of refractory material that does not react with the molten metal and has a relatively low thermal expansion so that it does not deform the coolerbody. The lower end of the insulator 144 extends slightly beyond the lower end of the die 122" and the coolerbody while it has an enlarged outer diameter to form a step 144' similar in function to the step 116 on the die 112. The upper end should be placed near the lower end of the casting zone, usually 12.5 mm below the upper edge of the bushing 118. If the upper end extends too high, relative to the outside insulator, the strand will cast against the insulator leaving indentations in the strand. The bore dimensions of the inside insulator are also significant, particularly on startup, during a hold, or during a slow down, because the melt begins to solidify on the inside insulator 144. To prevent termination, the inner surface of the insulator 144 must be smooth and tapered to widen upwardly. As with the die 112', the outside insulator or bushing 118 is used in conjunction with the inside insulatpr 144 to reduce the aforementioned difficulties.

Referring again to Fig. 4, a ceramic hat 146 surrounds the coolerbody 103 and the manifold extension assembly 102 to insulate them thermally from the metallic melt, so that the coolerbody may perform its function of cooling the mold so that rod solidification may occur. The hat 146 is formed from any suitable refractory material such as cast silica. The hat 146 attaches to the manifold 54 by means of a ring 148 which is spring biased against the manifold 54 by a spring 149. By this means of attachment, the hat 146 is pulled tightly against the coolerbody 103 while allowing for dimensional changes from differential thermal expansion. The spring 149 is preloaded to create a total force greater than the highest G loading to be experienced during oscillation, thereby maintaining a tight seal between the hat 146 and the coolerbody 103. The hat allows the mold assembly to be immersed in the melt to any preselected depth. While immersion to a level below the casting zone is functional, the extremely high production speed characteristics are, in part, a result of a relatively deep immersion. One advantage of this deep immersion is to facilitate feeding the melt to the liquid core of the casting in the casting zone. A vapor shield 150 and gaskets 151 (see also

Fig. 5) are placed in the gap between the hat and the coolerbody adjacent the die to prevent the melt and vapors from entering the gap and to further thermally- insulate the coolerbody. The gaskets are preferably three or four annular layers or "donuts" of the afore mentioned "Fiberfrax" refractory fiber material, while the vapor shield is preferably a "donut" of molybdenum foil interposed between the gaskets 151. The shield 150 and gaskets 151 extend from the die extension 112a to the outer diameter of the coolerbody. The combined thickness of these layers is sufficient to firmly engage the coolerbody face 103a and the end face of the hat 146 typically one-quarter inch.

In a typical cycle of operation, the casting furnace 16 is filled with a molten alloy. A rigid, stainless steel rod is used to start up the casting. A steel bolt is screwed into the lower end of the rod. The rod has the dimensions of the strand to be cast, e.g. 19 mm diameter rod, so that the rod can be fed down through the mold assembly and can be engaged by the withdrawal machine 22.

Whenever the mold assembly is inserted into the melt, cone of a material non-contaminating to the melt being cast, preferably solid graphite, covers the die portion 112a (or a refractory die extension such as the inside insulator 144). An additional alloy cone 48 of a material non-contaminating to the melt, typically copper, covers the lower end of the hat 146. The cones pierce the cover and dross on the surface of the melt to reduce the quantity of foreign particles caught under the coolerbody and in the die. The melt dissolves the cone 48 and the starter rod bolt pushes the smaller graphite cone off the die and it floats to the side. An advantage of the preferred form of this invention, utilizing a projecting die portion 112a, is that it supports and locates the smaller graphite cone on insertion into the melt. To function properly, the surface of the larger cone 48 should form an angle of forty-five degrees or less with the vertical.

After the graphite cone has been displaced, the bolt extends into the melt and the melt solidifies on the bolt. During start up and after the strands have advanced sufficiently above the drive wheels 44, the cast rod is sheared below the steel bolt and the strands are mechanically diverted onto the booms 24, 24'. Before replacing the starter rods in a storage rack for reuse, the short length of casting and the steel bolt is removed. An alternative starter rod design uses a short length of rigid stainless steel rod attached to a flexible cable which can be fed directly onto the boom 24 because of its flexibility. The withdrawal machine is then ramped up to a speed to being the casting. Between shifts or during temporary interruptions, such as for replacement of a coiler, the strand is stopped and clamped. Casting is resumed simply by unclamping and ramping up to full speed.

As the strand 12 is withdrawn, forward strokes pull the solidified casting formed in the casting or solidification zone upwardly to expose melt to the cooled die, which quickly forms a skin on this newly exposed die surface. During steady state operation, the rod is pulled at a constant rate in the range from 508 to 1016 cm/min. Simultaneously, the entire mold assembly, including the enclosed die 112, is oscillated vertically with an acceleration of about 1 g, reaching a top speed of about 10 cm/s in each direction. The oscillation allows the new skin to strengthen and attach to the previously formed casting. Because of the high cooling rate of the coolerbody and the steep temperature gradient generated by the outside insulator 118, the solidification occurs very rapidly over a relatively short length of the die. As stated earlier, typical melt temperatures for oxygen free copper and copper alloys are 1038 to 1260°C. In practicing the present invention, the insulator (bushing 118) insulate the melt from the coolerbody to maintain the melt as a liquid within the die below the casting zone. Near the upper edge of the insulator the melt temperature drops rapidly and solidification begins. In casting 19 mm brass rod at over 254 cm/min, the casting zone extends longitudinally for 2.54 to 3.84 cm. At the top of the casting zone, the strand is solid. Estimated average temperature of brass castings in the solidification zone are 899 to 954°C. A typical temperature for the brass casting as it leaves the mold assembly is 816°C. At the upper end of the mold assembly, there is a clearance around the strand to ensure the presence of oxygen or a water saturated atmosphere to burn off zinc vapors before they condense and flow down to the casting zone. The strand, thus produced, is of exceptionally good quality. The strand is characterized by a fine grain size and dendrite structure, good tensile strength and good ductility.

There has been described a simple, low cost oscillating mold assembly and a withdrawal process for use with the mold assembly that are capable of continuously producing high quality metallic strands, particularly brass, at extraordinarily high speeds. In particular, the mold assembly and withdrawal process provide sophisticated solutions to the many serious difficulties attendant the casting environment such as extreme temperatures and temperature differentials, metallic and water vapors, foreign particles present in the casting furnace and differentials in the thermal expansion coefficients of the materials forming the mold assembly.

The invention is further illustrated by the following non-limiting example.

Using the apparatus illustrated in Fig. 2 of the drawing, strand 12 was continuously cast from a melt of free-cutting brass, CDA 360. 1998 kg of the molten alloy was charged into furnace 16 and was maintained in the molten state. The composition for alloy CDA 360 is:

After initiating casting of a strand 12. by insertion of a pipe with a screw on its end through die 112 into the melt followed by withdrawal of the pipe in the manner known in this art, the solidified strand 12 was drawn by rollers 44 at a speed of 508 cm/min. At the initiation of continuous withdrawal of strand 12, the body 18 of the oscillating mold was immersed in the melt to a depth of about 12.7 cm. During casting, the dunk depth of body 18 varied from approximately 17.8 to 7.62 cm immersion. During mold oscillation, the temperature of the melt was maintained at 1010°C and molten alloy was fed into furnace 16 as needed during casting to maintain the immersion depths of body 18. The diameter of the die 15 was 0.75 inches to produce strand 12 with a diameter of about 19 mm. The forward and reverse mold speed during oscillation reached a top value of 10.2 cm/sec due to a mold acceleration of 1 g. The distance the mold travelled between its uppermost position in the melt and its bottommost position was approximately 4.4 cm. The temperature of strand 12 as it left the die 112 was approximately 816°C.

After casting, the rod was hot fabricated successfully. Cast grain size was from columnar, 1 mm. Wrought structure was fine recrystallized throughout the section (.025-.050 mm).

While the invention has been described with reference to its preferred embodiments, it will be understood that modifications and variations will occur to those skilled in the art. For example, while the die 112 has been described as extending the full length of the coolerbody 103, for many applications it can extend only a short distance above the casting zone.

## Claims

1. A method for continuously up-casting a metallic strand (12) from a metallic melt (14) comprising:
providing a vertically oriented die (112) having an inlet end (112a) with a coolerbody (103) having a free end portion surrounding a portion of said die (112) to enable portions of said die (112) to be cooled and with an insulating member (118) located within a recess in the coolerbody (103) and between a portion of said die (112) and a portion of said coolerbody (103) to insulate a portion of said die (112) from the cooling of said coolerbody (103), the inlet end (112a) of said die (112) extending substantially below the free end portion of said coolerbody (103), and the location of said insulating member (118) being at the free end portion of the coolerbody (103) extending between said die (112) and said coolerbody (103) a predetermined distance;
immersing said free end portion of said coolerbody into the melt (14) a distance greater than said predetermined distance to produce a solidification front (114a) within the die (112) when the melt (14) is withdrawn through said coolerbody (103);
withdrawing molten metal from the melt (14) through said die (112) while cooling said die (112) through said coolerbody (103), said cooling completely solidifying the molten metal into a strand (12) within a portion of the die (112) above the insulating member (118);
and providing alternating forward and reverse movements of the die (112) and the strand (12) relative to each other in a direction parallel to the direction of the travel of the strand (12);
characterized in that the solidified strand (12) is withdrawn from said melt (14) at a constant'rate;
and that said die (112) is oscillated in a direction parallel to the direction of travel of said strand (12).

2. The method as set forth in claim 1 wherein a cooling fluid is circulated through said coolerbody (103) to a point just above the top of the insulating member (118) to initiate solidification of the melt (14) into a strand (12) within the portion of the die (112) backed by said insulating member (118) and to completely solidify said melt (14) into a strand (12) within a portion of the die (112) above the insulating member (118).

3. The method as set forth in claim 2, wherein the part of said coolerbody (103) that is immersed in said melt (14) is protected from the heat of the melt (14) by an insulating material forming an insulating barrier (146) between the melt (14) and the coolerbody (103).

4. The method as set forth in claim 1, wherein said strand (12) is withdrawn from said die (112) with a withdrawal rate of 508 to 1016 cm/min.

5. The method as set forth in claim 4, wherein said die (112) oscillates with an acceleration of about 1 g in each direction reaching a top speed of about 10 cm/s.

6. The method as set forth in claim 5, wherein the frequency of oscillation is in the range of 12 to 150 cycles per minute.

7. Apparatus for continuously up-casting a metallic strand (12) from a metallic melt (14) according to the method claimed in claim 1, comprising:
a vertically oriented, generally tubular die (112) having an inlet end (112a) for fluid communication with the melt (14);
a coolerbody (103) having a free end portion (103a) surrounding a portion of said die (112) to enable portions of said die (112) to be cooled, the inlet end (112a) of said die (112) extending substantially below-the free end portion of said coolerbody (103);
an insulating member (118) located between a portion of said die (112) and said coolerbody (103) to insulate a portion of said die (112) from the cooling of said coolerbody (103), the location of said insulating member (118) being at said free end portion (103a) of the coolerbody (103) and extending between said die (112) and said coolerbody (103) a predetermined distance;
supporting means (20) mounted for immersing said free end portion (103a) of said coolerbody (103) in the melt (14) a distance greater than said predetermined distance to produce a. solidification front (114a) within the die (112) below the level of the melt (14) when the melt (14) and the solidified strand (12) is withdrawn through said die (112);
means (44) for withdrawing the melt (14) and the strand (12) through said die (112) while cooling said die through said coolerbody (103), said cooling completely solidifying the molten metal into said strand (12) within a portion of the die (112) below the level of the melt (14) and above the insulating member (118),
characterized in that the solidified strand (12) is withdrawn from said melt (14) at a constant rate by the withdrawing means (44); and that
oscillating means (225) are provided for oscillating said die (112) in a vertical direction parallel to the direction of travel of said strand (12) in a pattern of forward and reverse strokes.

8. Apparatus as set forth in claim 7, wherein a cooling fluid is circulated through said coolerbody (103) to a point just above the top of the insulating member (118) to initiate solidification of the melt (14) into a strand (12) within the portion of the die (112) backed by said insulating member (118) and to completely solidify said melt (14) into a strand (12) within a portion of the die (112) above the insulating member (118).

9. Apparatus as set forth in claim 7, wherein the height of said melt (14) is continuously adjusted with respect to said coolerbody (103).

10. Apparatus as set forth in claim 9, wherein the height of said melt (14) is adjusted by an elevator which rises in response to a signal related to the weight of the melt.

## Revendications

1. Procédé de coulée ascendante ou en source continue d'un fil ou brin métallique (12) au départ d'une masse fondue métallique (14) comprenant:
la prévision, pour une filière (112) orientée verticalement et comportant une extrémité d'entrée (112a), d'un corps refroidisseur (103) présentant une partie extrême libre entourant une portion de cette filière (112) pour permettre le refroidissement de parties de la filière (112), ainsi que d'un élément isolant (118) localisé dans une cavité du corps refroidisseur (103) et entre une partie de la filière (112) et une partie du corps refroidisseur (103) afin d'isoler une partie de cette filière (112) du refroidissement du corps refroidisseur (103), l'extrémité d'entrée (112a) de la filière (112) s'étendant sensiblement en dessous de la partie extrême libre du corps refroidisseur (103), et la localisation de cet élément isolant (118) se situant à la partie extrême libre du corps refroidisseur (103), cet élément s'étendant entre la matrice (112) et le corps refroidisseur (103) sur une distance prédéterminée;
l'immersion de la partie extrême libre susdite du corps refroidisseur dans la masse fondue (14) sur une distance supérieure à la distance prédéterminée susdite pour produire un front de solidification (114a) à l'intérieur de la filière (112) lorsque la masse fondue (14) est extraite à travers le corps refroidisseur (103);
l'extraction de métal fondu depuis la masse fondue (14) à travers la filière (112), tandis que cette filière (112) est refroidie par le corps refroidisseur (103), ce refroidissement solidifiant totalement le métal fondu en un fil (12) dans une partie de la matrice (112) se situant au-dessus de l'élément isolant (118);
et la prévision de déplacements alternés vers l'avant et vers l'arrière de la filière (112) et du fil (12) l'un par rapport à l'autre dans une direction parallèle à la direction de déplacement du fil (12);
caractérisé en ce que le fil solidifié (12) est extrait de la masse fondue (14) à une vitesse constante, et en ce que la filière (112) est amenée à osciller dans une direction parallèle à la direction de déplacement du fil (12).

2. Procédé suivant la revendication 1, caractérisé en ce qu'un fluide de refroidissement est mis en circulation à travers le corps refroidisseur (103) vers un point se situant juste au-dessus de haut de l'élément isolant (118) pour amorcer une solidification de la masse fondue (14) en un fil (12) dans la partie de la filière (112) entourée par l'élément isolant (118) et pour solidifier totalement la masse fondue (14) en un fil (12) dans une partie de la filière (112) se situant au-dessus de l'élément isolant (118).

3. Procédé suivant la revendication 2, caractérisé en ce que la partie du corps refroidisseur (103) qui est plongée dans la mass fondue (14) est protégée de la chaleur de cette masse fondue (14) par un matériau isolant formant une barrière isolante (146) entre la masse fondue (14) et le corps refroidisseur (103).

4. Procédé suivant la revendication 1, caractérisé en ce que le fil (12) est retiré de la filière (112) à une vitesse d'extraction de 508 à 1016 cm/ mn.

5. Procédé suivant la revendication 4, caractérisé en ce que la filière (112) oscille avec une accélération d'environ 1 g dans chaque direction, en atteignant une vitesse supérieure d'environ 10 cm/s.

6. Procédé suivant la revendication 5, caractérisé en ce que la fréquence d'oscillation se situe dans l'intervalle de 12 à 150 cycles par minute.

7. Appareil pour la coulée en source ou ascendante continue d'une fil ou brin métallique (12) au départ d'une masse fondue métallique (14) suivant le procédé de la revendication 1, comprenant:
une filière (112) d'allure générale tubulaire, orientée verticalement et comportant une extrémité d'entré (112a) destinée à être mise en communication avec la masse fondue (14);
un corps refroidisseur (103) comportant une partie extrême libre (103a) entourant une portion de la filière (112) pour permettre le refroidissement de parties de cette filière (112), l'extrémité d'entrée (112a) de la filière (112) s'étendant sensiblement en dessous de la partie extrême libre du corps refroidisseur (103);
un élément isolant (118) localisé entre une partie de la filière et le corps refroidisseur (103) pour isoler une partie de cette filière (112) du refroidissement du corps refroidisseur (103), et la localisation de cet élément isolant (118) se faisant à la partie extrême libre (103a) du corps refroidisseur (103) en s'étendant entre la filière (112) et ce corps refroidisseur (103) sur une distance prédéterminée;
un dispositif de support (20) monté pour l'immersion de la partie extrême libre (103a) du corps refroidisseur (103) dans la masse fondue (14) sur une distance supérieure à la distance prédéterminée susdite pour créer un front de solidification (114a) à l'intérieur de la filière (112) en dessous du niveau de la masse fondue (14) lorsque cette masse fondue (14) et le fil solidifié (12) sont extraits à travers la filière (112);
des moyens (44) pour l'extraction de la masse fondue (14) et du fil (12) à travers la filière (112), tandis que celle-ci est refroidie par le corps refroidisseur (103), ce refroidissement solidifiant totalement le métal fondu pour former le fil (12) dans une partie de la filière (112) se situant en dessous du niveau de la masse fondue (14) et au dessus de l'élément isolant (118),
caractérisé en ce que le fil solidifié (12) est extrait de la masse fondue (14) à une vitesse constante par les moyens d'extraction (44), et en ce qu'un dispositif d'oscillation (225) est prévu pour faire osciller la filière (112) dans une direction verticale parallèle à la direction de déplacement du fil (12) suivant un programme de courses vers l'avant et vers l'arrière.

8. Appareil suivant la revendication 7, caractérisé en ce qu'un fluide de refroidissement est mis en circulation à travers le corps refroidisseur (103) jusqu'en un point se situant juste au dessus du haut de l'élement isolant (118) pour amorcer la solidification de la masse fondue (14) en un fil (12) à l'intérieur de la partie de la filière (112) entourée par l'élément isolant (118), et pour solidifier complètement cette masse fondue (14) en un fil (12) dans une partie de la filière (112) se situant au dessus de l'élément isolant (118).

9. Appareil suivant la revendication 7, caractérisé en ce que la hauteur de la masse fondue (14) est réglée de manière continue par rapport au corps refroidisseur (103).

10. Appareil suivant la revendication 9, caractérisé en ce que la hauteur de la masse fondue (14) est réglée par un dispositif élévateur qui s'élève en réponse à un signal qui est en rapport avec le poids de la masse fondue.

## Patentansprüche

1. Verfahren zum kontinuierlichen Aufwärtsgießen eines Metallstrangs (12) aus einer Metallschmelze (14), welches umfaßt:
Es wird eine vertikal ausgerichtete Kokille (112) mit einem Einlaßende (112a) mit einem Kühlkörper (103) versehen, der einen freien Endbereich hat, der einen Teil der Kokille (112) umgibt, um die Kühlung von Teilen der Kokille (112) zu ermöglichen, wobei ein Isolationselement (118) in einer Aussparung des Kühlkörpers (103) und zwischen einem Teil der Kokille (112) und einem Teil des Kühlkörpers (103) angeordnet ist, um einen Teil der Kokille (112) gegen die Kühlung durch den Kühlkörper (103) zu isolieren, wobei sich das Einlaßende (112a) der Kokille (112) bis deutlich unterhalb des freien Endbereichs des Kühikörpers (103) erstreckt und wobei das Isolationselement (118) am freien Endbereich des Kühlkörpers (103) angeordnet ist und sich zwischen der Kokille (112) und dem Kühlkörper (103) über eine vorgegebene Strecke erstreckt;
der freie Endbereich des Kühlkörpers wird in die Schmelze (14) auf einer Strecke eingetaucht, die größer ist als die vorgegebene Strecke, um eine Erstarrungsfront (114a) innerhalb der Kokille (112) zu erzeugen, wenn die Schmelze (14) durch den Kühlkörper (103) abgezogen wird;
das geschmolzene Metall wird aus der Schmelze (14) durch die Kokille (112) abgezogen, während die Kokille (112) durch den Kühlkörper (103) gekühlt wird, wobei diese Abkühlung das geschmolzene Metall innerhalb eines oberhalb des Isolationselements (118) liegenden Bereichs der Kokille (112) vollständig zu einem Strang (12) erstarren läßt;
und es werden alternierende Vorwärts- und Rückwärtsbewegungen der Kokille (112) und des Stranges (12) relativ zueinander und parallel zur Laufrichtung des Stranges (12) herbeigeführt;
dadurch gekennzeichnet, daß der erstartte Strang (12) aus der Schmelze (14) mit einer konstanten Geschwindigkeit abgezogen wird, und daß man die Kokille (112) parallel zur Laufrichtung des Stranges (12) oszillieren läßt.

2. Verfahren gemäß Anspruch 1, bei dem man durch den Kühlkörper (103) eine Kühlflüssigkeit bis zu einem Punkt zirkulieren läßt, der gerade oberhalb des oberen Endes des Isolations- elementes (118) liegt, um das Erstarren der Schmelze (14) zu einem Strang (12) in einem Bereich der Kokille (112) einzuleiten, welcher durch das Isolationselement (118) abgestützt wird, und um die Schmelze (14) in einem oberhalb des Isolations-elementes (118) liegenden Teil der Kokille (112) vollständig zu einem Strang (14) erstarren zu lassen.

3. Verfahren gemäß Anspruch 2, bei dem der Teil des Kühlkörpers (103), der in die Schmelze (14) eingetaucht wird, gegen die Hitze der Schmelze (14) durch ein Isolationsmaterial geschützt ist, welches eine isolierende Sperre (146) zwischen der Schmelze (14) und dem Kühlkörper (103) bildet.

4. Verfahren gemäß Anspruch 1, bei dem der Strang (12) aus der Kokille (112) mit einer Abzugsgeschwindigkeit von 508 bis 1016 cm/min abgezogen wird.

5. Verfahren gemäß Anspruch 4, bei dem die Kokille (112) in jeder Richtung mit einer Beschleunigung von etwa 1 g oszilliert und dabei eine Höchstgeschwindigkeit von etwa 10 cm/s erreicht.

6. Verfahren gemäß Anspruch 5, bei dem die Oszillationsfrequenz in dem Bereich von 12 bis 150 Zyklen pro Minute liegt.

7. Vorrichtung zum kontinuierlichen Aufwärts-Gießen eines Metallstrangs (12) aus einer Metallschmelze (14) nach dem in Anspruch 1 beanspruchten Verfahren, umfassend:
Eine vertikal ausgerichtete, im wesentlichen rohrförmige Kokille (112) mit einem Einlaß (112a) für ein (Flüssigkeits-)Kommunizieren mit der Schmelze (14);
einen Kühlkörper (103) mit einem freien Endbereich (103a), welcher einen Teil der Kokille (112) umgibt, um das Abkühlen von Teilen der Kokille (112) zu ermöglichen, wobei das Einlaßende (112a) der Kokille (112) sich bis deutlich unterhalb des freien Endbereichs des Kühlkörpers (103) erstreckt;
ein Isolationselement (118), welches zwischen einem Teil der Kokille (112) und dem Kühlkörper (103) angeordnet ist, um einen Teil der Kokille (112) gegen die Kühlung durch den Kühlkörper (103) zu isolieren, wobei das Isolationselement (118) an dem freien Endbereich (103a) des Kühlkörpers (103) angeordnet ist und sich über eine vorgegebene Strecke zwischen der Kokille (112) und dem Kühlkörper (103) erstreckt;
Stützeinrichtungen (20), die so montiert sind, daß der freie Endbereich (103a) des Kühlkörpers (103) in die Schmelze (14) auf einer Strecke (mit einer Länge) eintaucht, die größer ist als die vorgegebene Strecke, um eine Erstarrungsfront (114a) innerhalb der Kokille (112) unterhalb des Pegels der Schmelze (14) zu erzeugen, wenn die Schmelze (14) und der erstarrte Strang (12) durch die Kokille (112) abgezogen werden;
Einrichtungen (44) zum Abziehen der Schmelze (14) und des Stranges (12) durch die Kokille (112), während die Kokille (112) durch den Kühlkörper (103) gekühlt wird, wobei durch das Kühlen ein vollständiges Erstarren des geschmolzenen Metalls zu einem Strang (12) in einem Teil der Kokille (112) herbeigeführt wird, der unter dem Pegel der Schmelze (12) und über dem Isolationselement (118) liegt,
dadurch gekennzeichnet, daß der erstartte Strang (12) durch die Abzugseinrichtung (44) aus der Schmelze (14) mit einer konstanten Geschwindigkeit abgezogen wird und daß Oszilliereinrichtungen (225) vorgesehen sind, um eine oszillierende Bewegung der Kokille (112) in vertikaler Richtung und parallel zur Laufrichtung des Stranges (12) in einer Folge von Vorwärts- und Rückwärtshüben herbeizuführen.

8. Vorrichtung gemäß Anspruch 7, bei der man eine Kühlflüssigkeit durch den Kühlkörper (103) bis zu einem Punkt unmittelbar über dem oberen Ende des Isolationselementes (118) zirkulieren läßt, um das Erstarren der Schmelze (14) zu einem Strang (12) in dem Teil der Kokille (112) einzuleiten, der durch das Isolationselement (118) abgestützt wird, und um die Schmelze (14) in einem oberhalb des Isolationselementes (118) befindlichen Teil der Kokille (112) vollständig zu einem Strang (12) erstarren zu lassen.

9. Vorrichtung gemäß Anspruch 7, bei der die Höhe der Schmelze (14) kontinuierlich bezüglich des Kühlkörpers (103) eingestellt wird.

10. Vorrichtung gemäß Anspruch 9, bei der die Höhe der Schmelze (14) mittels einer Hubvorrichtung eingestellt wird, die in Abhängigkeit von einem Signal steigt, welches mit dem Gewicht der Schmelze verknüpft ist.
